

## UNITED STATES PATENT OFFICE

SHINJIRO HORII, OF TOKYO, JAPAN

## BACKING FOR STENCIL SHEETS

No Drawing. Application filed February 21, 1928, Serial No. 256,061, and in Japan January 23, 1928.

My invention relates to backing sheet for stencil sheets commonly used for autographic and type-writing duplication.

The backing sheets commonly used are 5 made of firm, stiff paper, on which are superimposed stencil sheets of fibrous base, e. g., Japanese yoshino paper, coated with a material impermeable to ink.

It has been proposed to provide a backing 10 sheet of firm paper the face of which is covered with printing ink with a color contrasting sharply with the color of the superimposed stencil sheet. In that case, the characters cut upon the stencil sheet are more visible to the typist. And again, the face of the 15 backing sheet is most efficient as an extractor, the small particles of wax expressed from the fibers of the base of the stencil sheet by the impact of the type clinging to such printed 20 backing sheet.

It has also been proposed to provide a backing sheet of firm paper having a varnished surface, which serves the double purpose of 25 making the sheet impervious to moisture and of acting as an adhesive for the purpose of binding a soft absorbent paper firmly thereto.

The backing sheet, in accordance with the 30 present invention, consists of a firm paper impregnated with a coating material chiefly 25 consisting of non-drying oil, e. g., castor oil, or a similar oil, either with or without a hardening material, such as waxes or resins. While this backing sheet may be used in combination with any kind of stencil sheet, it is 35 most suitable for use with the so-called dry-process stencil sheet which has a coating including a gelatinous organic colloid, such as gelatine, or esters of polysaccharides, dispensed with an oleaginous softening material.

40 It has been found that a backing sheet which has a coating of drying oils or varnishes, as above referred to, has a certain disadvantage in that the coating is not stable and, therefore, will not keep long as it absorbs 45 oxygen from the air, or sticks together with the coating of the stencil sheet due to the presence of resins which react with the oleaginous materials.

The backing sheet, according to this invention, has a coating chiefly of non-drying

oil, it has a grease-proofing quality and is very stable, so that it will keep a long time. Moreover, it does not become hard and brittle as in the case where drying oils or varnishes are used, and does not stick to the surface of a stencil sheet. 55

In the practice of the invention a firm stiff, paper, such as manila paper, is coated on one or both sides with a coating material composed largely of non-drying oil, e. g., castor 60 oil, and if desired a hardening material, e. g., as carnauba wax, Montan wax, bees wax, copal, ester gum, or a mixture of these the substances being previously dissolved in a suitable solvent such as turpentine oil, benzol, 65 petroleum benzine or a mixture of them. And then the coated sheet after the evaporation of the volatile matter may be calendered through hot rollers.

70 By way of illustration, although the proportions of the ingredients of the coating material may vary according to circumstances, an example is given as follows:

|                   | Example | Parts by weight | 75 |
|-------------------|---------|-----------------|----|
| Castor oil        | -----   | 90              |    |
| Carnauba wax      | -----   | 5               |    |
| Copal             | -----   | 5               |    |
| Turpentine oil    | -----   | 100             | 60 |
| Benzol            | -----   | 200             | 80 |
| Petroleum benzine | -----   | 100             |    |

It has heretofore been suggested to employ a backing sheet in combination with a stencil sheet of the type which should previously be moistened, the backing sheet being impregnated with glycerine and water. It has also been suggested to provide a backing sheet impregnated with a composition containing glycerine, Turkey-red oil, water and a coloring material. These backing sheets are used for the purpose of uniformly softening a hygroscopic stencil sheet and to retain the moistening material, keeping the backing sheet for a long period of time in 85 usable condition. However, according to the present invention, the backing sheet being stiff, firm and grease-proof only serves as a protection against the dissipation of 90 the oils contained in the coating of the so- 95 100

called dry-process stencil sheet which does not require any moistening, but it produces even and clear characters on the stencil sheet. Turkey-red oil is a salt of sulphonated glycerides of fatty acids, and therefore, is not included in the present invention.

The stencil sheet is superimposed upon the backing sheet and the former may be attached at one end to the latter as in the usual 10 way.

In the stencil-cutting operation, the combined stencil and backing sheet is introduced into the typewriting machine and the characters are produced on the stencil sheet by 15 the impact of the type of the machine, or the sheet may be stencilized by the pressure of a hand stylus in the usual manner. It results in a sharply defined clear copy. It is more convenient to insert a sheet of thin 20 paper, or cloth, immediately between the stencil sheet and the backing sheet for the sake of producing even characters on the stencil sheet.

What I claim is:—

- 25 1. A backing sheet for a dry-process stencil sheet consisting of a firm stiff paper treated with a coating composition including a non-drying oil and a hardening material for the purposes described.
- 30 2. A backing sheet for a dry-process stencil sheet consisting of a firm stiff paper treated with a coating composition including a non-drying oil, waxes and resins for the purpose described.

35 In testimony whereof I affix my signature.  
SHINJIRO HORII.

40

45

50

55

60